

10/12  
Patented Mar. 12, 1940

2,193,346

## UNITED STATES PATENT OFFICE

2,193,346

## MOLDED PRODUCT

Allan B. Ruddle, San Francisco, Calif.

No Drawing. Application December 10, 1937,  
Serial No. 179,150

5 Claims. (CL 22-188) ✓

This invention relates to molded products, and particularly to a composition for molding which has as its principal ingredient sand or other similar granular or powdery substance.

5 The present application is a continuation in part of my copending application entitled "Molded product", Serial No. 165,765, filed September 25, 1937. The said copending application describes a method for and product of molding 10 from sand and the like for manufacturing various articles, and particularly for making foundry cores for metal casting purposes.

The present invention relates particularly to such cores. The cores used in foundry practice 15 are usually constructed of ordinary molded sand with ingredients added to facilitate molding the sand to a definite shape, and permit baking or curing the core to render it sufficiently hard or firm to stand up under the pouring of molten metal, yet friable enough to be readily broken out of the completed casting.

The object of the present invention is to provide a molded article particularly adapted for use 20 as a foundry core which is formed entirely of relatively inexpensive materials, and to provide 25 a core which, although having exceptional resistance to breakage by the pouring against it of molded metals, will upon cooling or setting of the metal be so easily broken that it will readily return to its granular or sand-like form.

30 A further object of the invention is the provision of a core that will be capable of drying or being cured very rapidly, and a core in which the drying and effect of drying will be uniform throughout.

35 Another object is the provision of a core having a minimum tendency to stick or adhere to the mold or core box to which it is formed.

I have discovered, as set forth in my copending 40 application above referred to, that a satisfactory molded core may be made by mixing with common molding sand an alkali metal silicate, an alkali metal fluosilicate, and either an acid or an alum. It is preferred that the materials used 45 for this purpose be such as are available at relatively low cost. Sodium silicate and sodium fluosilicate meet this requirement and are typical of the alkali metal silicates and fluosilicates that may be used. Aluminum sulphate is an example of an inexpensive alum-like substance that 50 is suitable for the purpose of the present invention. In making cores, I first prepare a solution in the proportions of about

55 2 gallons water  
1-10 ounces aluminum sulphate  
1-10 ounces alkali fluosilicate, and  
1-10 gallons of an alkali metal silicate

60 The solution made within the limits of the above formula should be a clear liquid of approximate-

ly 30° to 32° Baumé. One part by volume of this solution is then mixed with from 5 to 60 parts of common molding sand, depending upon the use for which the product is being made.

5 I have discovered further that certain qualities of the cores made according to the above prescribed practice may be greatly improved by slight variations in the proportions of the materials set forth above, and by the addition thereto of a bitumen, preferably emulsified such, for example, as an emulsion of asphalt.

I have also discovered that the use of a bituminous emulsion such as an emulsion of asphalt in combination with the above solution in making a sand core has several advantages. It makes 15 a core that will break up readily after it has been used. This is an important feature of the manufacture of cores, because where cores are made sufficiently durable to withstand the effect of molten metal being poured against them, they 20 are in some cases so hard that it is difficult to remove the core from the casting after the casting has cooled. Easy removal of the core is particularly important in cases where the core forms small or irregular passages in the casting such, 25 for example, as the water jacket or block in the cylinder head of an internal combustion engine. In making such a casting with cores made in accordance with the present invention, the cores have not only stood up under pouring in a manner which compares favorably with the finest 30 cores made by other methods, but after cooling of the casting, a slight jar is sufficient to so completely break up the core that it may be poured from the casting in a finely divided granular 35 condition.

40 A further advantage of cores made according to the present invention is that they may be dried or cured very quickly without harmful results. For example, cores having a wall thickness of approximately two inches may be completely cured by an exposure to a temperature of about 500° F. for a period of fifteen minutes or less. The presence of the bituminous emulsion in the core also effects a uniformity in the curing process in that a core made in this manner is found to dry with a uniform hardness throughout, whereas the same core with the emulsion omitted has a tendency to dry or cure harder in some parts than in others, and usually harder in the lower regions of the core, which is probably due to the fact that the binding materials used with the sand have a tendency to drain toward or collect at the bottom of the core before 55 it is completely cured. The asphalt also produces the very desirable result of preventing adherence of the core to the box or form in which it is molded so that the production of a perfect core is made more easy by the elimination of 60

the danger of breaking away parts of the core as it is removed from the core box.

The following formula is cited as typical of proportions used in practising the present invention, but the exact proportions given are not to be taken as actual nor as limiting the scope of the invention:

1750 c. c. dry sand.  
125 c. c. of a solution of approximately:  
2 gallons water  
1-10 ounces aluminum sulphate  
1-10 ounces alkali fluosilicate, and  
1-10 gallons of an alkali metal silicate  
40 c. c. of an asphalt emulsion  
65 c. c. of water

In mixing, the emulsion is preferably first added to the solution and thoroughly stirred and then the water is added, the stirring being continued to insure thorough mixing and distribution of the emulsion and the solution. The resulting liquid is added to the sand in a manner to impart an even distribution of moisture and uniform molding qualities to the sand. Where the sand is to be used is not perfectly dry, the water in the mixture may be reduced slightly to obtain the same ultimate result.

I have referred to sand as one ingredient of my core, and it should be understood that the term "sand" as used herein in the appended claims is any type of molded sand or other granular material capable of being used in this manner.

35 The invention as described above pertains to  
molded cores of all types used in foundry prac-  
tice and similar practices.

Having thus described my invention, what I claim and desire to secure by Letters Patent is—

1. A molded product comprising sand and a binder of an alkali metal silicate, an alkali metal fluosilicate, aluminum sulphate, and a bituminous emulsion. 5

2. A molded product comprising a mixture of sand, a binder which consists principally of about

**2 gallons of water**

1-10 ounces of aluminum sulphate  
1-10 ounces of an alkali metal fluosilicate  
1-10 gallons of an alkali metal silicate

and a bituminous emulsion.

3. A molded product comprising a mixture of 15 sand, a binder which consists principally of about

2 gallons of water  
1-10 ounces of aluminum sulphate  
1-10 ounces of sodium carbonate

1-10 ounces of sodium fluosilicate  
1-10 gallons of sodium silicate 20

and a bituminous emulsion.

2. A molded product comprising sand, a liquid binder and an asphalt emulsion, said liquid binder comprising an aqueous solution obtained by combining aluminum sulfate and an alkali metal fluosilicate with a large excess of an aqueous solution of a water soluble silicate. 25

5. A molded product comprising sand, a liquid binder and an asphalt emulsion, said liquid binder comprising an aqueous solution obtained by combining an alkali metal fluosilicate with a large excess of an aqueous solution of a water soluble silicate.

ALLAN B. BUDDLE 25